

## UNITED STATES PATENT OFFICE

MICHAEL GEORGE CORSON, OF NEW YORK, N. Y., ASSIGNOR TO THE DURIIRON COMPANY, INC., OF DAYTON, OHIO, A CORPORATION OF NEW YORK

## PROCESS OF TREATING IRON-SILICON ALLOYS

No Drawing. Application filed May 9, 1928, Serial No. 276,502. Renewed February 20, 1932.

The invention relates to iron-silicon alloys and to a process of treating same. In particular, the invention relates to the treatment of iron-silicon alloys containing upwards of 5% silicon to render them workable and impart ductility thereto.

It has been known for a long time that iron-silicon alloys become practically unforgeable when the silicon content is raised above about 5%. However, the alloys containing higher percentages of silicon possess certain properties, namely high electric resistivity and resistance to corrosion, which, if combined with ductility, would render them desirable for various uses.

I have found that the brittleness of the iron-silicon alloys is due to two causes. The first is that silicon forms with iron a compound  $Fe_3Si$  which is characterized by hardness and lack of ductility. Therefore, when the silicon is added to pure iron in increasing proportion up to 14.4% silicon the alloys change from a very ductile metal to an unwieldy compound. This entails a continuous decrease in ductility and increase in hardness.

Secondly, all these alloys have to pass through a double transformation when cooling from the casting temperature. At temperatures included between 1400° C. and 1040° C., the actual temperature at which the transformation begins depending on the composition and varying as to the upper limit inversely with the proportion of silicon, these alloys begin to change from a uniform solid solution, the delta phase, to a duplex structure of delta plus gamma the main body of each grain becoming enriched with silicon.

At temperatures ranging from 900 to 1040° C. the alloys go through an opposite transformation which, if the temperature is maintained within the desired range a sufficient length of time, changes the metal back into a uniform solid solution. If such time is not allowed, the retransformation to the condition of a uniform solid solution remains incomplete and this incompleteness, in addition to the weakness or brittleness due to the presence of the duplex structure, causes ad-

ditional weakness of the grains along their slip planes. It is for these reasons that the tendency of these alloys to break under every effort of forging or rolling is to be attributed. The ingots cooling down in the molds do not have time enough to pass evenly and completely through the two transformations. Cooling of the incompletely transformed ingots causes them to develop ultramicroscopic cracks and these do not weld together when the ingots are reheated for forging.

Accordingly, my process aims to so conduct the casting, cooling and working of the metal as to insure completion of the double transformation and to prevent the formation of ultramicroscopic cracks in the metal and the development of a structure causing brittleness and lack of strength.

I have also found that nickel, when present in small amounts, not exceeding 1%, and usually less than .5%, acts as a catalyst during the two transformations described, thereby accelerating the rate of transformation and substantially shortening the time during which the temperature of the metal is to be closely controlled, as well as further improving the ductility and workability of the metal. The invention, therefore, includes as a modification the addition of small amounts of nickel for the purpose above mentioned.

The invention comprises broadly the casting, cooling and working, either by forging or rolling, of iron-silicon alloys containing upwards of 5% and preferably not exceeding about 14.4% silicon, under such conditions as will insure the absence of transformations and prevent the appearance of a duplex structure during the process of working. The invention further includes the cooling of alloys of the class above-described, either after working above the two transformation zones or directly from the casting operation without working at such a rate and under such conditions as to insure the retransformation to a uniform solid solution or delta phase of the delta plus gamma structure which may have formed when passing through the first transformation zone, thereby preventing the

55

60

65

70

75

80

85

90

95

100

development of a structure causing brittleness and lack of strength.

The metal may be cooled from the casting temperature sufficiently slowly when passing through the temperature ranges at which the respective transformations take place to insure completion of each transformation before cooling to a lower temperature, thereby producing a uniform solid solution. Or, since it is not essential that the first transformation,—from delta to delta plus gamma,—shall have been permitted to become complete before the retransformation to delta phase or a uniform solid solution begins, the metal in cooling may be passed either slowly or quickly through the range at which the first transformation takes place so long as it is held for a sufficiently long time in the range where the second transformation takes place to insure its completion. The metal may then be reheated and worked to the desired extent. Since cooling of the metal from the casting temperature to the cold condition under the above conditions requires a relatively long controlled heat treatment, usually at least 24 hours, it is found more feasible from a practical standpoint, to carry out the working of the metal before the ingots have cooled to below the working temperature. The necessity for reheating is also thereby eliminated.

According to a preferred procedure for carrying out the invention, an iron-silicon alloy of any desired composition within the range specified is prepared, preferably under conditions insuring the absence of carbon in the product. The molten alloy is poured into molds preheated preferably to at least 850° C. or to such a temperature as will insure that the outer portions of the ingot will not have become chilled to a point where the first formation will begin before the ingot has become solid enough to be removed from the mold. As soon as the ingot has solidified sufficiently to be removed from the mold, it is placed in a furnace and subjected to a soaking treatment while maintaining the temperature of the furnace above the temperature at which the first transformation begins until the temperature throughout the ingot has become equalized. For example, when treating a 12% silicon alloy the furnace temperature should be above about 1050° C. When treating alloys containing between 6 and 11% silicon the furnace temperature preferably should be about 100° higher or above approximately 1150° C.

The metal is permitted to remain in the furnace until it is desired to start the working operation, when the ingot is immediately rolled or forged while hot. The temperature of the metal during working preferably should not be permitted to fall to the point where the first transformation begins, although a slight under cooling may take

place without detriment providing the transformation is quickly checked by reheating. Therefore, the temperature of the metal at the beginning of the working operation should be considerably above the minimum soaking temperatures above-mentioned in order to allow for cooling during working and if considerable work is to be performed upon the metal it may require reheating treatments between successive working steps to insure the maintenance of an optimum working temperature of the metal as above-indicated. After its shape has been changed by the application of mechanical work to the desired degree, the worked material is returned to the furnace which is closed completely and the temperature lowered by small steps until a temperature of 500° C is reached. This procedure renders the alloy reasonably ductile at low temperature so that the drop in ductility is much less pronounced than that observed in iron-silicon alloys produced in the normal way as the silicon content increases from the substantially pure iron to the  $Fe_3Si$  compound.

The cooling of the metal at a controlled rate after the working operation is important, particularly through the range at which the second transformation will take place; since this second transformation proceeds slowly. However, as it continues far below its point of beginning its completion may be insured and the cooling of the metal expedited by cooling the wrought metal through such range gradually and at such a rate that such transformation will have become completed when the temperature has dropped to the point where the transformation will no longer take place. I have ascertained this point to be about 500° C. with iron-silicon alloys of the class above-mentioned. Good results are insured by cooling these alloys from 900 to 500° C. in approximately 12 hours.

As indicated above, I have found that nickel in small amounts from about 0.2% to 1%, and usually less than .5%, acts as a catalyst during the two transformations described, thereby shortening the heat treatment considerably and effecting improvement in the properties of the alloy. Accordingly, I prefer to introduce small amounts of nickel into the alloy, although it is not essential that nickel be added in order to produce a marked improvement in the ductility and workability of the alloy.

I have indicated above that it is preferable to produce the alloy under conditions that insure the absence of carbon in the resulting product, owing to the bad influence of carbon on the workability of alloys of the type here considered. However, in certain cases it may be desirable to use a carbon-containing scrap in making the alloy. I have found that the best way to eliminate the bad

influence of carbon is to introduce a metal with which it will combine in the presence of silicon to form coalesced carbides instead of films and flakes of graphite. Most carbide-forming elements tend in the presence of silicon to stay in solid solution in the iron. I have found, however, that vanadium forms carbides in the presence of silicon and that when it is present in small amounts up to 10 1% the properties of the carbon-containing alloys are substantially improved due to conversion of the carbon into the carbide form. When approximately 1% of vanadium is present it will eliminate as much as 15% 15 carbon by converting it into carbide.

It will be understood that various changes may be made in the details of the procedure outlined and in the composition of the alloy without departing from the invention which 20 is not to be deemed as limited other than as indicated in the appended claims.

What I claim is:

1. Process of making wrought articles of an iron-silicon alloy containing upwards of 25 5% silicon which comprises casting said alloy into a mold preheated to at least 850° C., removing the resulting ingot from said mold when it has cooled sufficiently to be self-sustaining and before transformation of the 30 metal from a state of solid solution has taken place, soaking said ingot at a temperature of at least 1050° C., working said ingot to produce articles of the desired form and size while maintaining the temperature thereof 35 above the point where ultramicroscopic cracks begin to develop on rapid cooling, and finally gradually lowering the temperature to a point where rapid cooling does not affect the properties of the metal.

2. Process of making wrought articles of an iron-silicon alloy containing upwards of 5% silicon which comprises casting and then working said alloy to the desired form and size without permitting the same to cool below about 1040° C. at any time between casting and completion of the working step, and then cooling gradually to a point where rapid cooling does not materially affect the properties of the metal.

3. Process of making wrought articles of an iron-silicon alloy containing upwards of 5% silicon which comprises casting and then soaking and working said alloy to the desired form and size without permitting the same to cool below about 1040° C. at any time between casting and completion of the working step, and finally cooling gradually to a point where rapid cooling does not materially affect the properties of the metal.

4. Process of producing a workable iron-silicon alloy containing upwards of 5% silicon which comprises casting the alloy into a mold preheated to at least 850° C., then immediately after removing the resulting metal from the mold bringing it to a substantially

uniform temperature throughout of at least 1050° C., and then cooling to a point below 900° C. at a sufficiently low rate as to substantially prevent the formation of ultramicroscopic cracks.

5. Process of producing a workable iron-silicon alloy containing upwards of 5% silicon which comprises casting the alloy in a preheated mold, removing the resulting ingot from the mold before it has cooled below the 70 point at which the uniform solid solution—the delta phase—starts to change to a duplex structure of delta plus gamma, heating the metal while still heated as aforesaid at above 1050° C. and then cooling at a sufficiently 75 slow rate as to substantially prevent the formation of ultramicroscopic cracks.

6. Process of producing wrought articles of iron-silicon alloys containing from 6 to 11% silicon which comprises casting the 80 alloy, removing the resulting ingot from the mold before it has cooled below the point where the uniform solid solution begins to change to a duplex structure of delta plus gamma, then without further cooling heating the metal at above 1150° C. to effect structural homogenization, working the metal while maintaining the temperature thereof sufficiently high to prevent formation of the duplex structure and finally cooling the resulting wrought articles, the rate of cooling through the range 900° C.-500° C. being so adjusted as to insure completion of retransformation to a uniform solid solution of the 85 delta plus gamma structure formed during 90 cooling.

7. Process of improving the ductility and workability of iron-silicon alloys containing upwards of 5% silicon which comprises adding nickel in small amounts up to 1%, casting the alloy in a mold preheated to at least 850° C., removing the resulting ingot from the 105 said mold when it has cooled sufficiently to be self-sustaining, then heating said ingot at a temperature of at least 1050° C. until the structural homogenization which takes place above said temperature has become complete and then cooling the metal sufficiently slowly to below 900° C. as to insure that the metal 110 is brought into a state of substantially uniform solid solution.

8. Process of making wrought articles of iron-silicon alloys containing upwards of 5% silicon which comprises forming an alloy containing iron and silicon in the desired proportions, adding vanadium in sufficient amounts to convert any carbon present to the form of a carbide, casting the alloy, removing the resulting ingot from the mold when it has cooled sufficiently to become self-sustaining, heating the ingot to effect equalization of the temperature thereof, and working the metal, the temperature of the metal 120 throughout the casting, cooling, heating and

working steps being maintained above about 1040° C.

9. Process of improving the ductility and workability of iron-silicon alloys containing upwards of 5% silicon which comprises forming an alloy containing iron and silicon in the desired proportions, adding vanadium in small amounts up to 1% to convert any carbon present to the form of carbides, casting the alloy, removing the resulting ingot from the mold when it has cooled sufficiently to become self-sustaining, then heating the ingot at a temperature above the point where transformation from the delta phase to delta plus gamma begins, to effect structural homogenization of the metal, and then cooling, the rate of cooling through the range at which retransformation of the delta plus gamma structure to a uniform solid solution will take place being so controlled as to insure completion of such retransformation.

10. Process of improving the ductility and workability of iron-silicon alloys containing upwards of 5% silicon which comprises forming an alloy containing iron and silicon in the desired proportions, adding vanadium in sufficient amount to convert any carbon present to the carbide form, casting the alloy in a mold preheated to at least 850° C., removing the resulting ingot from the mold when it has cooled sufficiently to become self-sustaining, then heating the ingot to at least 1050° C. until the structural homogenization which takes place above said temperature has become complete, and then cooling the metal sufficiently slowly through the range 900° C.-500° C. to insure conversion of any delta plus gamma structure formed during previous stages into a state of substantially uniform solid solution.

11. Process of improving the ductility and workability of iron-silicon alloys containing upwards of 5% silicon which comprises casting the alloy into a heated mold, removing the resulting ingot from the mold before the temperature thereof has dropped to 900° C., heating the ingot to at least 1050° C. and then hot working.

12. A wrought metal article consisting principally of iron and containing from 5% to about 14% silicon, and characterized by a physical structure and properties such as are produced when an alloy of like composition is cast in a mold preheated to at least 850° C., removed while hot, and then soaked and worked to the desired form and size without permitting the same to cool below about 1040° C., followed by gradual cooling to a point below 900° C.

13. A metal article consisting principally of iron and containing from 5% to about 14% silicon, and characterized by a physical structure and properties such as are produced when an alloy of like composition is cast in a preheated mold, removed from the

mold before it is cooled below the point at which the uniform solid solution starts to change to a duplex structure of delta plus gamma, then heated at above 1050° C. to effect structural homogenization, followed by gradual cooling to a point below 900° C.

In testimony whereof, I have signed my name to this specification this 3rd day of May, 1928.

MICHAEL GEORGE CORSON.

75

80

85

90

95

100

105

110

115

120

125

130